

Oct. 16, 1951

J. E. WALTZ

2,571,975

MELT SPINNING PROCESS

Filed May 10, 1947



INVENTOR.  
*Joseph Elmer Waltz*  
BY  
*C. H. Mortenson*

ATTORNEY

## UNITED STATES PATENT OFFICE

2,571,975

## MELT SPINNING PROCESS

Joseph Elmer Waltz, Wilmington, Del., assignor  
to E. I. du Pont de Nemours & Company, Wil-  
mington, Del., a corporation of Delaware

Application May 10, 1947, Serial No. 747,252

18 Claims. (Cl. 18—54)

1

This invention relates to the spinning of nylon yarn and more particularly to the production of yarn of uniform properties by spinning the yarn by a process which controls the troublesome depolymerization of the polymer which occurs at spinning temperatures.

Commercial nylon is a synthetic linear condensation polyamide formed by the condensation of suitable monomers or low molecular weight polymers with the elimination of water. Consequently, water is normally present in the flake prior to spinning, the water being either a portion of that formed during polymer production or an amount absorbed from the surrounding atmosphere. It is well-known that at elevated temperatures the degree of depolymerization of polyamides is a function of the amount of water present. To avoid excessive degradation by water steps are usually taken to dry the polymer flake to a low and controlled moisture content prior to the melt spinning step. In addition to using flake containing only small amounts of free moisture, steps may be taken to sweep away some of the water present during spinning by conducting the spinning in a moving atmosphere of very dry nitrogen or other suitable gas. By such means it is possible to obtain a satisfactory polymer. However, in the spinning of nylon yarn, a small inventory of polymer melt is maintained in the spinning cell for a short interval of time prior to its passing to the metering pump and then to the spinneret. The processes of polymerization and depolymerization can proceed during this melted stage and, without control, yarn is produced having variable molecular weight, and hence variable tenacities, elongations, dyeing characteristics and other non-uniform properties. While the polymer is standing in the melt stage it is virtually impossible to remove all the moisture and to keep operating conditions constant. Thus, the amount and kind of nitrogen used, the unit temperatures maintained, the gas pressures and similar conditions vary considerably. Because of the critical nature of these known processes it is extremely difficult to produce a yarn having optimum uniformity of physical properties.

Accordingly, it is an object of this invention to provide a process which avoids the difficulties referred to above and which results in yarn of high quality and uniform properties. A further object is the provision of means for controlling the polymerization-depolymerization equilibrium. A still further object is the provision of a process by which yarn having very good uniformity

2

may be obtained without the use of costly materials such as highly purified nitrogen or a similar gas. Other objects will appear hereinafter.

These objects are accomplished by the following invention in which spinning is conducted under a positive and predetermined water vapor pressure. The nylon polymer flake is melted in the presence of water vapor, the water vapor pressure being controlled. The melt is then spun without subjecting it to temperature variations or changes in water vapor pressures. In practice, the polymer flake is melted in the presence of steam the pressure of which is controlled. The melt is allowed to stand for a brief period until equilibrium is reached and it is then metered and spun under conditions which keep the effect of the steam constant.

This invention will be more clearly understood by reference to the attached Figure 1 which is a diagrammatic, side elevation view of a suitable melt spinner.

In Figure 1, in which like numbers refer to like parts, the polymer is fed into the melt spinner through the polymer flake supply duct 10. The flake passes down through the open hopper 11 into a preheater 12. This preheater is heated in any convenient way, as, for example, by means of a steam jacket 13. Steam is passed into the heated jacket at 14 and is passed to the trap at the bottom of the heater at point 15. At point 16 a portion of the steam is removed and is sent through the bypass 17 in which is located a valve 18. The flake after being preheated passes downward to point 19 at which it comes into contact with the steam passing through valve 18. The steam delivered to the preheater jacket 13 is preferably high pressure steam (10-100 pounds per square inch) and thereby provides a temperature of the order of 115 to 170° C. The steam that passed through valve 18 is at atmospheric pressure at point 19 since the hopper 11 is open to the atmosphere. Operation in this manner provides an automatic control of steam pressure and it is possible to keep the pressure in the melt spinner within very narrow limits. The polymer melt is in equilibrium with steam and, accordingly, the viscosity of the melt is uniformly controlled. The steam introduced into the flake at point 19 passes up through the polymer flake and out into the air at point 20. Thus, the steam serves to blanket the polymer and to adjust the viscosity of the melt in relation to the water vapor pressure of the steam.

56 After mixing with the steam, the flake passes

to a grid melter 21 which may be heated by steam or electricity or other means. The polymer becomes thoroughly melted and forms a melt pool 22. Polymer is then metered out through the pump 23 which passes the melt in fixed and constant amount to the spinneret assembly 24. The inventory of polymer in the melt 22 is kept as small as possible in order to prevent decomposition. It is, however, preferred to keep an amount sufficiently large enough so that the polymer after melting stands exposed to the steam for a minimum of about 15 minutes before being metered out. This exposure permits establishment of an equilibrium.

In the conventional nitrogen processes the amount of water in the melt ranges from 0.11% to 0.18% even under the most rigid control. Further, the water vapor pressure varies from 550 mm. to 850 mm. of Hg. This variation results in yarn non-uniformities as mentioned above. By the process of this invention it has been found possible to maintain a constant amount (0.16% for polyhexamethylene adipamide) of moisture in the melt, and a more constant pressure (710-770 mm. of Hg) in the cell. This constancy in moisture content results in an accurately controlled polymerization-depolymerization equilibrium and the spun polymer has physical properties which are much more uniform than comparable polymer spun by the conventional nitrogen processes.

The amount of water in the melt will depend, among other factors, upon the polyamide being spun. Thus, while the amount is 0.16% for polyhexamethylene adipamide, the figure for other polyamides may be substantially higher or lower. The important point is that for each polymer being spun by the process of this invention, the amount of water in the melt remains constant during spinning and does not vary between certain limits prevailing when the particular polyamide is melt spun by conventional processes. Similarly, the pressure in the spinning unit will depend, in part, upon its location or, in other words, the local atmospheric conditions. In general, the maximum fluctuations will be  $\pm 30$  mm. of Hg. The main point is that the pressure in the spinning unit during spinning by the process of this invention will be very nearly equal to the atmospheric pressure. Since the atmospheric pressure at a given location generally fluctuates only  $\pm 30$  mm. of Hg, the pressures in the spinning cells will be substantially constant. As pointed out above, by the process of this invention the fluctuation in pressure within the cell is advantageously maintained within narrow limits.

The advantages obtainable by use of the process of this invention may be seen by comparing the physical properties of yarn produced by the process of this invention to the physical properties of yarn produced by conventional spinning methods using purified nitrogen as the atmosphere over the melt pool. The examples which follow are given for illustrative purposes and are not to be considered as limitative. In the standard process using polyhexamethylene adipamide and a nitrogen pressure of 20 pounds per square inch, a yarn was produced having an average tenacity of 4.59 grams per denier with an overall standard deviation of 0.234. When the same polymer was spun by the process of this invention the yarns had a comparable average tenacity (4.43 grams per denier) but the overall standard deviation was considerably lower, being only 0.148. Similarly, polyhexa-

methylene adipamide after spinning showed for the yarn spun by the process of this invention a relative viscosity of 26.0 (8.4% solution of polymer in formic acid) with an overall standard deviation of only 0.53. Comparable polymer spun by the conventional spinning methods had a similar average relative viscosity (27.7) but a much higher overall standard deviation of 1.04. This shows that the polymer spun by the process of this invention had a more uniform molecular weight than the polymer resulting after spinning by the standard spinning method using nitrogen as the atmosphere over the melt pool.

In addition to greater uniformity in molecular weight and in tenacities, the yarns of this invention had greater uniformity in elongations. The average elongation figures for the yarn spun by the process of this invention was 24.0% as compared to an average elongation of 22.1% for yarn spun in a similar manner by the conventional process. The average standard deviations for the two yarns, however, were 2.28 and 2.42, respectively, showing the greater uniformity in this respect of the yarns of this invention.

These advantages in uniformity disclosed are summarized in the following table:

TABLE I

| Yarn       | Property         | Standard Deviation |
|------------|------------------|--------------------|
| Control    | Molecular Weight | { 1.04             |
| Steam Spun |                  | 0.53               |
| Control    | Tenacity         | { 0.234            |
| Steam Spun |                  | 0.148              |
| Control    | Elongation       | { 2.42             |
| Steam Spun |                  | 2.28               |

Further, the acid-dye variations for the yarns of this invention are surprisingly low both in number and severity. More level coverage was obtained in the dyeing of yarns of this invention than in the dyeing of yarns produced by the conventional practice. This can be seen in Table II below which is based on severity ratings involving the number and depth of dye-junctions observed per 100 yards of woven fabric. Ratings shown in the table vary from a rating of 1, a barely discernible junction, to a rating of 12, a very severe junction.

TABLE II

*Dye junctions in 100-yards of woven fabric*

| Depth               | Number of Junctions |            |
|---------------------|---------------------|------------|
|                     | Control             | Steam-Spun |
| 1                   | 18                  | 67         |
| 2                   | 27                  | 43         |
| 3                   | 13                  | 6          |
| 4                   | 17                  |            |
| 5                   | 4                   |            |
| 6                   | 4                   |            |
| 7                   | 2                   |            |
| 8                   | 7                   |            |
| 10                  | 14                  |            |
| 12                  | 28                  |            |
| Rating <sup>1</sup> | 729                 | 171        |

<sup>1</sup> Summation of the product of the number of junctions per 100 yards of fabric and the depth of each.

From the above table it can be seen that the acid-dye variations for the yarn of this invention are only one-fourth as great as in control yarn. In other words the dye coverage of steam spun yarn with acid-dye is about four times better than the coverage in the acid-dyed controlled fabric. Prior to this invention the variation in physical and chemical properties of the yarn pre-

cluded the commercial use of acid-dyes and it was necessary to rely upon the use of acetate dyes. The process of this invention produces a yarn having physical and chemical properties the uniformity of which permits the use of acid-dyes, the dyed products being equivalent in uniformity to commercial nitrogen-spun yarns dyed with acetate dyes. The commercial use of acid-dyes is desirable since a greater variety of dyed products may be produced through the use of this additional class of dye-stuffs.

While the yarns in the above examples were prepared using dry steam at atmospheric pressures, steam at higher pressure may be used. The steam pressure may be as high as 30 pounds per square inch gauge but generally it is preferred to use steam pressure within the limits of 7 to 10 pounds per square inch gauge. The maximum steam pressure which can be used is dependent upon factors such as the nature of the polyamide being spun, and the type of yarn being formed. In general, the higher the steam pressure the higher is the amount of water in the melt in equilibrium with the steam. The higher the pressure of the water vapor the lower is the viscosity of the melt. Further, when high pressure steam is employed, it is usually necessary to preheat the polymer flake in order to reduce the condensation of moisture on the flake which would otherwise form. Operation at pressures appreciably below atmospheric pressure is also possible. When using the higher pressures mentioned above or reduced pressures, closed systems are required.

Thus, it is preferred to use dry steam at atmospheric pressure because the process is much simpler. High pressure apparatus is not needed. Further, the steam when used at atmospheric pressure does not tend to keep steam and gases of decomposition dissolved in the polymer to the extent that steam under pressure does. Further, a free flowing, controlled volume of steam passing over the melted polymer and through the flakes in the preheater provides a satisfactory means for eliminating occluded air.

While the process of this invention has been described in particular reference to polyhexamethylene adipamide, many other synthetic linear polyamides may be used. For example, the following may be mentioned: polytetramethylene-adipamide, polytetramethylenebacamide, polypentamethyleneadipamide, polypentamethylenebacamide, polyhexamethylene - adipamide, polyhexamethylenebacamide, polyhexamethylene-ene-glutaramide, polyoctamethyleneadipamide, poly - p - xylylenesbacamide, and the polyamide derived from 3,3' - diaminodipropyl ether and adipic acid. Polymerized epsilon-amino-caproic acid, polymerized 9-aminononanoic acid, and polymerized 11-amino-undecanoic acid are examples of linear polymers, derived from amino acids, which may also be used. Further, copolyamides or interpolyamides and any mixtures of polyamides may be spun, by the process of this invention to form yarns of high quality. In general any polyamide, which includes the polyesteramides, may be used, such as are described in U. S. 2,071,250, U. S. 2,071,253, U. S. 2,130,523, U. S. 2,130,948 and U. S. 2,190,770. While a specific melt spinner has been described this invention is not limited thereby and any equivalent or similar device may be used.

By the process of this invention it has been found possible to use polymer flake of moisture content as high as 6.5%. Contrary to the present

practice of the industry, it is not required in the working of this invention to use polymer flake of low and controlled moisture content. This is a matter of considerable importance since the process becomes more economical. Generally, it is preferred to use flake which has reached equilibrium with ordinary atmospheric conditions. Such flake contains about 4% moisture. No great or costly effort is necessary to condition the flake prior to spinning such as, for example, conditioning in atmospheric pressure of controlled humidity. Generally, mere exposing flake to normal atmospheric conditions is adequate. This is a marked advantage since no special equipment is required.

The results of the process of this invention are surprising and contrary to the literature and expectation of one skilled in the art. Since moisture plays an important role in the degradation of nylon held at elevated temperatures, it would appear unlikely that yarn of uniform and satisfactory properties could be obtained by melt spinning the polymer under a positive water vapor pressure and in the presence of considerable amounts of water vapor. However, as shown above, it has been found that this can be done by the process of this invention which provides yarn of the desirable quality in a surprisingly simple manner. Yarn having very uniform properties in respect to tenacity and elongation and dye depths and having high and uniform molecular weights is produced by the process of this invention. The necessity of using equipment for operating under a positive pressure of nitrogen gas (20 pounds per square inch) is eliminated. Thus, the process is freed of many problems of equipment, design construction and operation. It is also freed from the required maintenance of feeding locks and storage locks and the repeated purging of them in order to remove air. The operation of this invention does not require carefully predried flake nor large volumes of purified gas as an inert atmosphere. The criticalness which the standard methods for spinning under nitrogen required is eliminated by the process of this invention. It is much easier to control the water vapor pressure in the process of this invention which involves the use of only one gaseous material (steam) than in the conventional processes which involve the use of two gases (water vapor and nitrogen). Surprisingly and advantageously, yarn of the greater uniformity is produced in a practicable manner and with a reasonable requirement of criticalness.

Any departure from the above description which conforms to the present invention is intended to be included within the scope of the claims.

I claim:

1. A process for spinning a synthetic linear polyamide which comprises melting the said polyamide in a chamber; introducing water vapor into said chamber at a substantially atmospheric pressure; exposing the resultant melted polyamide to the said water vapor until water is uniformly distributed in the melt; and feeding the resultant molten composition to a means for extruding it from said chamber, the melting and the feeding being carried out at substantially atmospheric pressure and in the presence of water vapor at substantially constant pressure.

2. A process for spinning a synthetic linear polyamide which comprises melting the said polyamide in a chamber; introducing water vapor into said chamber at substantially atmospheric

pressure; exposing the resultant melted polyamide to the said water vapor until water is uniformly distributed in the melt; and feeding the resultant molten composition to a means for extruding it from said chamber, the melting and feeding being carried out at substantially atmospheric pressure at a substantially constant vapor pressure of water and the said molten composition having a substantially constant moisture content prior to extrusion.

3. In a process for melt spinning a synthetic linear polyamide the steps comprising melting said polyamide in a chamber; introducing into said chamber water vapor at substantially atmospheric pressure; exposing the resultant melted polyamide to the said water vapor until water is uniformly distributed in the melt; and feeding the said polyamide to a means for extruding it from the said chamber, said melting and feeding being carried out at substantially atmospheric pressure and in the presence of a substantially constant vapor pressure of water.

4. In a process for melt spinning a synthetic linear polyamide, steps comprising melting said polyamide in the presence of a water vapor at substantially atmospheric pressure, said vapor being introduced into said chamber; exposing the resultant molten composition to said vapor until water is uniformly distributed in the said molten composition; and feeding the said molten composition to a means for extruding it from said chamber, the said steps being carried out at substantially atmospheric pressure.

5. A process in accordance with claim 1 wherein the said polyamide is polyhexamethylene-adipamide.

6. A process in accordance with claim 1 wherein said polyamide is polyhexamethylenesebacamide.

7. A process in accordance with claim 1 wherein in said polyamide is polymerized epsilon-amino-caproic acid.

8. A process for spinning a synthetic linear polyamide which comprises melting said polyamide in a chamber; introducing water vapor at substantially atmospheric pressure into said chamber; exposing said polyamide to said vapor which is in the form of steam substantially at atmospheric pressure; allowing the resultant molten composition to come into equilibrium with said water vapor so that water is uniformly distributed in said molten composition; and feeding said molten composition at substantially atmospheric pressure and in the presence of said water vapor to a means for extruding it from said chamber.

9. A process for spinning a synthetic linear polyamide which comprises melting said polyamide in a chamber; introducing water vapor into said chamber at a pressure of from 710 to 770 mm. of mercury; exposing said polyamide to said water vapor; allowing the resultant molten composition to come into equilibrium with said water vapor so that water is uniformly distributed in said molten composition; and feeding said molten composition at a pressure of from 710 to 770 mm. of mercury and in the presence

of said vapor to a means for extruding it from said chamber.

10. A process for maintaining the rate of polymerization and rate of depolymerization at equilibrium in a molten synthetic linear polyamide which comprises heating, at substantially atmospheric pressure, said polyamide in an atmosphere consisting of water vapor at substantially atmospheric pressure until water is uniformly distributed in said polyamide.

11. A process in accordance with claim 10 in which said pressure is from about 710 to about 770 mm. of mercury.

12. A process in accordance with claim 10 wherein said polyamide is polyhexamethylene-adipamide.

13. A process in accordance with claim 10 wherein said polyamide is polyhexamethylene-sebacamide.

14. A process in accordance with claim 10 wherein said polyamide is polymerized epsilon-amino-caproic acid.

15. A process for spinning a synthetic linear polyamide which comprises melting the said polyamide in a chamber the atmosphere of which consists of water vapor; introducing the water vapor into said chamber at a substantially constant pressure of up to 10 pounds per square inch gauge; exposing the molten polyamide to said water vapor until water is uniformly distributed throughout the molten polyamide; and feeding the resultant molten composition to a means for extruding it from said chamber, the said melting and the said feeding being carried out in the said atmosphere consisting of said water vapor.

16. A process for keeping the rate of polymerization occurring in a molten synthetic linear polyamide equal to the rate of depolymerization occurring in said polyamide which comprises heating said polyamide in an atmosphere consisting of water vapor at a pressure of up to 10 pounds per square inch gauge until water is uniformly distributed throughout said polyamide.

17. A process in accordance with claim 16 in which said heating is carried out for at least 15 minutes.

18. A process in accordance with claim 1 in which the polyamide is polyhexamethylene adipamide and the amount of water uniformly distributed therein is about 0.16%.

JOSEPH ELMER WALTZ.

#### REFERENCES CITED

The following references are of record in the 55 file of this patent:

#### UNITED STATES PATENTS

| Number    | Name    | Date           |
|-----------|---------|----------------|
| 2,253,176 | Graves  | Aug. 19, 1941  |
| 2,295,942 | Fields  | Sept. 15, 1942 |
| 2,303,340 | Dreyfus | Dec. 1, 1942   |

#### OTHER REFERENCES

Maxness: "Preheating with Steam," Plastics, February 1947, pages 34-36, 39, 90.